

Feb. 2, 1932.

A. SCHUBERT

1,843,741

TRANSFER PRINTING PROCESS FOR LEATHER

Filed May 9, 1930



INVENTOR.

*Alfred Schubert*  
BY *George Kinsella & Co., Inc.*  
his ATTORNEYS.

## UNITED STATES PATENT OFFICE

ADOLF SCHUBERT, OF MILLBURN, NEW JERSEY, ASSIGNOR TO BARRETT & COMPANY, OF NEWARK, NEW JERSEY, A CORPORATION OF NEW JERSEY

## TRANSFER PRINTING PROCESS FOR LEATHER

Application filed May 9, 1930. Serial No. 451,196.

This invention relates to the application to the marking of leather, of a transfer-printing process that I have developed for making permanent markings on fibrous articles and which is peculiarly suited for ornamentation work. The present invention concerns protecting the leathers against a deleterious action which the chosen dye solvent may have.

Hereinafter, for simplicity of expression, 10 I shall frequently refer to ink as incorporating a single dye (singular number); it will be understood however, that any given ink may contain two or more dyes.

In this process, the subject matter (letters, 15 numerals, lines, masses of colors, pictures, etc., etc.) is laid down in an ink containing an undissolved dyestuff or dyestuffs, and then the dyestuff is transferred to the article or material ultimately intended to receive the 20 marking by contact in the presence of a transfer agent, so-called, which is or includes a solvent for the dyestuff or dyestuffs, and which solvent is capable, or is made capable, of permeating the vehicle portion of the ink. 25 Sheets of paper, cloth, or the like, on which the subject matter may be printed and from which the transfer is thus made, are called "transfer sheets".

In applying my process thus briefly outlined to the ornamenting of leather, I use as 30 the dyestuff in the ink a dye capable of dyeing leathers or skins, rather than, for example, a discharge, mordant or resist, and it frequently happens that a desired solvent for the dye, 35 used in transferring the dye to the leather, is a substance that has a deleterious action on the leather. For example, the alcohols, and particularly ethyl alcohol, are desirable substances for use as the dye solvent in making 40 the transfer to leathers; ethyl alcohol however has a deleterious action on the vegetable tanned leathers and some of the chrome tanned leathers; it tends to extract the tannin.

45 The object of the present invention is to avoid this deleterious action, and this I now propose to do by so treating the leather that a compound, substantially insoluble in the transfer agent, is formed with the tannic acid 50 on or in the fibres of the leather. Preferably

the compound formed is one which is transparent or colorless; that is to say, the compounds should be transparent or colorless except where opacity or color may not be objectionable. To form such an insoluble compound with the tannic acid, ethyl alcohol being used as the dye solvent, calcium and barium salts are preferred; particularly calcium bromide and barium bromide; and most preferably calcium bromide.

55 In applying my present invention therefore: I use as the ink, one incorporating a dye capable of directly dyeing the leather to be worked on (using the term "dye" with the meaning hereinafter given to it), and usually 60 an alcohol-soluble dye. With the chosen dye, there is mixed a vehicle to suit the particular conditions under which the subject matter is laid down for transfer of the dye to the leather, as suiting the particular printing 65 process selected for printing on paper sheets; thus for printing on sheets of paper, cloth or other similarly light thin flexible materials, the vehicle material is so chosen that the ink resulting from the mixture has that viscosity, 70 tacky or greasy nature, or whatever other characteristics may be required of the ink used in the particular printing process employed for laying down the ink on the sheet.

75 Furthermore, I choose for the vehicle a substance or substances that will remain on such transfer sheets until the transfers are made to the leather; I believe that the presence of the vehicle at the time the transfer is made helps to confine the dye to its intended boundaries. The dye is not to be held in the vehicle in solution however, but in a solid state; in suspension as it were. If the dye-stuff is soluble in the vehicle, bleeding may 80 take place in the transfer sheet and this result in blurred outlines and poor color gradations in the reproduction on the leather. Furthermore, for certain colors, I have 85 seemed to find it impossible to get sufficient dye into the vehicle in dissolved form to give 90 the desired colored intensity in the reproduction. Hence I use as the vehicle portion of the ink (including in that term everything in the ink excepting the dye), a material or materials in which the dye is substantially 95 100

soluble. Conceivably the dye may be introduced into the vehicle initially in the form of a solution, if desired, provided the solvent is evaporated later for example, or if the 5 dye is precipitated or is otherwise restored to or produced in a solid state prior to printing on the transfer sheet base; at the time of the printing of the transfer sheet however, substantially all the dye should be in an undissolved state, but it should remain in this 10 solid state until the time for making the transfer to the leather. Preferably therefore, I take the dye in powdered form and grind it into the chosen vehicle. Afterwards 15 this mixture can be thickened if too thin, or thinned if too thick, by the addition of suitable inert substances as will be understood; also drying retardants and/or other useful substances can be incorporated in and made a 20 part of the ink as desired, and as will be understood.

With such an ink I usually print up a stock of transfer sheets at one time; that is to say, I print the subject matter on such a quantity of sheets of paper, cloth or other relatively light thin flexible material as may correspond to the number of skins or pieces of leather to be marked, or as may be needed for some time to come. Preferably I use a 30 fibrous material for these transfer sheet bases, because of the permeability of the fibrous materials. Newsprint paper is suitable and usually gives better results than a heavily sized paper. The stock of transfer 35 sheets can be used as needed so long as the subject matter remains clear and the vehicle remains on the transfer sheets and remains permeable to the dye solvent employed at the time of the transfer, or remains in a condition where it can be made permeable to the 40 dye solvent.

To make a transfer or print on a leather the ink is brought into contact with the leather, as by pressing one of the transfer 45 sheets smoothly to the leather, inked face to the leather, in the presence of a solvent or solvents of the dye. Preferably the solvent or solvents for the dye are chosen from those substances that have a high degree of capillarity with respect to the leather to be marked, and the particular kind of leather to be marked; that is to say, preferably the 50 dye solvent or solvents is or are a substance or substances which penetrates and diffuses rapidly through the particular leather to be marked, as explained in a co-pending application for patent, Serial No. 448,434, filed April 29, 1930. In addition, the solvent or solvents for the dye must enter readily into 55 the vehicle part of the ink, and be capable of carrying dye, or the needed dyeing principle from well within the vehicle into dyeing relation with the fibres of the leather. In order that the dye solvent may enter the vehicle, the 60 materials composing the vehicle and the dye 65

solvent (or one of the latter) may be so chosen with respect to each other that the dye solvent has this characteristic of and by itself; for example, the dye solvent may be a solvent for the ink vehicle also. In the alternative, an 70 additional substance may be employed to give the dye solvent access into the vehicle; the latter is the subject of a co-pending application of mine, Serial No. 448,435, filed April 29, 1930; the additional substance, say a solvent 75 for the vehicle, can be applied separately to the ink, or as a mixture with the dye solvent or solvents. Where the dye appears in the ink as a compound needing to be broken up, or which can be broken up, before its action on 80 the fibres is accomplished, (for example where the dye is in the form of a lake), the dye solvent can be selected for its ability to break up the compound, as well as dissolve the dye; or in the alternative, an additional 85 substance may be used, say along with the dye solvent, to break up the compound; the dye solvent need not then be a solvent for the dye compound found in the ink; it only need be a solvent for the dye proper, or the essential principle needed for dyeing the leather. 90 Usually I apply the dye solvent to the leather, either by spraying or dipping immediately before the transfer, and apply the transfer sheet direct to the wetted leather. 95 When two or more solvents are used, and also when an additional substance is to be used at the time of making the transfer, such for example as a substance to give the dye solvent or solvents access into a vehicle into which it 100 or they are otherwise substantially impermeable, I usually mix the whole and apply the mixture in the same way. Usually, too, I press the transfer sheet to the leather with considerable pressure, as in a press, in order 105 to evenly and uniformly contact the transfer sheet with the leather, the latter ordinarily varying considerably in thickness throughout its extent; I have used up to 300 lbs. per square inch. This is not to be understood to 110 indicate, however, that such high pressures as this are always necessary. Heat may be used simultaneously, as by passing steam through pipes provided in the plates of the press; heat is not altogether an essential however. The transfer of dye to the leather takes 115 place rather quickly, at least under high pressure, a transfer of an adequate quantity of dye being produced in from a fraction of a minute to two minutes. The length of time 120 the transfer sheet is left in contact with the leather does not seem to be critical however; for example, without heat I have left a transfer sheet in contact with a leather under pressure, for as much as five minutes without 125 producing noticeable bleeding or blurring. When the transfer has been accomplished, the transfer sheet is peeled off the leather of course. Preferably, I employ dye solvents 130 that are also volatile, so that they are readily

removed or escape naturally from the leather by evaporation after having performed their functions. For general use on leather I prefer the alcohol-soluble dyes, and as the dye solvent employed in making the transfer, I prefer ethyl alcohol, denatured or not.

Where the chosen dye solvent or dye solvents have a deleterious affect on the leather chosen to be marked, by converting or otherwise extracting a substance therefrom, as ethyl alcohol tends to affect the tannin in vegetable tanned leathers and some chrome tanned leathers, I propose (according to the present invention) to avoid this deleterious action by applying to the leather, as mentioned before, a substance which forms a compound with the substance attacked by the dye solvent, which compound is insoluble in the dye solvent or solvents, and, preferably, which is transparent or colorless. The time and manner of the application of this substance to the leather is not material, generally speaking.

Solids can be applied in the form of solutions. The protective substance or substances may be applied separate and apart from the transfer agent, or separate and apart from some of the substances used at the time of transfer when a multiple substance is employed in effecting the transfer: for example, the protective substance or substances may be applied to the leather before the dye solvent is applied to the leather, when the dye solvent is applied to the leather itself rather than to a transfer sheet. Preferably, however, the protective substance or substances is or are mixed with the dye solvent, for example, dissolved in the dye solvent, and the two applied as a unit.

It will now be apparent that various kinds of dyes can be used in the ink, and the exact nature of the dye employed is not material to my invention, excepting only that it be a dye capable of dyeing the leather, as the term "dyeing" is used in the dyeing art, and not a mere fixing of pigment to the leather by the vehicle of the ink after the manner of printing. The "dye" may be a substance capable as a whole of dyeing the leather, or it may be a compound, such as a lake, from which the dyeing principle is to be extracted; the matter of lakes has been mentioned above. For developed colors, or other dyes acting in analogous ways, all of the constituents may be incorporated in the ink when the conditions are suitable, or only a part of the constituents may appear in the ink and when necessary the remainder applied directly to the leather either before or after the transferring operation. In general, the various forms which the "dye" may assume will be understood by those skilled in the art, who will understand also the various manners in which the leather may be treated, either before or after the transferring is done, or both

before and after, to "prepare" the leather, for cleaning, to brighten the colors, etc., etc.

A specific example of my process incorporating the present invention, is illustrated in the accompanying drawings: In finely powdered form, alcohol-soluble Cochineal G. D. is ground into a rosin oil varnish, and the mixture may be thickened or thinned with otherwise inert substances, to such a consistency that the resulting dye-vehicle mixture has that consistency required for the operation of printing the transfer sheets. The ratio of the dye to the vehicle is found by trial, that ratio being used which gives the desired color strength or tintorial value of the leather. With the ink thus formed, the design or ornamental matter is printed on sheets of such paper as is used for news print, using blocks or rolls etched or engraved, or otherwise marked in accordance with the desired design, as the printing process may demand. Usually I print up a stock of these transfer sheets at once, since this ink will remain permeable to the dye solvent hereafter specified for quite awhile. For the transfer agent, I employ a saturated solution of ethyl alcohol, denatured or not, and calcium bromide, when transferring to a leather containing tannin subject to attack by the alcohol. When it comes time to make a transfer to, say, a vegetable tanned leather, the leather is sprayed with or dipped into the saturated solution of ethyl alcohol and calcium bromide, and immediately thereafter one of the transfer sheets is laid on the leather, inked face to the leather, and the two pressed momentarily in a press to evenly and uniformly contact the transfer sheet with the leather; a rather soft pad may be imposed between the transfer sheet and the adjacent plate of the press to aid this action. The rosin oil vehicle of the ink being soluble in the ethyl-alcohol, the ethyl alcohol penetrates well into the ink immediately upon this contact, dissolves more or less of the dye, and carries the same into the midst of the fibres of the leather to which it thereupon becomes affixed; that is to say, dyes the leather. Furthermore, on the application of the alcohol-calcium-bromide solution to the leather, the calcium bromide, entering the leather along with the alcohol, forms with the tannic acid of the leather a compound which is insoluble in the alcohol, so that the leather is protected against the deleterious action of the latter. After pressing the transfer sheet to the leather for a moment, the two are taken from the press and the transfer sheet is peeled off.

It will be understood from the foregoing that my invention is not limited to the details of the foregoing description, except as appears hereafter in the claims. Furthermore, it will be understood that when I use the word "compound" in describing the action between tannin and the protective substance or

substances, I am using this word "compound" in a rather broad sense, for example as including lakes, rather than in the narrow sense with which this word "compound" is sometimes used in chemistry in describing chemical reactions.

I claim:

1. In the method of making markings on leather, which consists in producing the subject matter in an ink incorporating a dye capable of dyeing the leather and vehicle material suiting the particular process by which the ink is laid down, and in which vehicle the dye is substantially insoluble, and pressing the subject matter, formed by such ink, to the leather in the presence of a solvent for the dye capable of carrying dye from the ink into the midst of the fibres of the leather, the improvement, where a substance used at the time of making the transfer to the leather has a deleterious affect on the leather, which consists in applying to the leather a material capable of forming with the part of the leather attacked by such substance, a compound on which said substance used at the time of transfer has substantially no affect.

2. In the method of making markings on leather, which consists in printing the subject matter on transfer sheet bases with an ink incorporating an alcohol-soluble dye for the leather and a vehicle material suiting the ink to the particular printing process by which the printing onto the transfer sheet bases is done, and in which vehicle the dye is substantially insoluble, and pressing, while the ink vehicle is still present on the transfer sheet, a transfer sheet to the leather in the presence of alcohol, the improvement, where the alcohol tends to affect tannin in the leather, which consists in subjecting the leather to a substance forming a compound with the tannin which is insoluble in the alcohol.

3. In the method of making markings on leather which consists in printing the subject matter on transfer sheet bases with an ink incorporating an alcohol-soluble dye for the leather and vehicle material suiting the ink to the particular printing process by which the printing onto the transfer sheet bases is done and in which vehicle substantially all the dye exists in an undissolved state, and pressing, while the ink vehicle is still present on the transfer sheet, a transfer sheet to the leather in the presence of alcohol, the improvement, where the alcohol tends to have a deleterious affect on the leather by attacking tannin therein, which consists in having present also, when the transfer sheet is pressed to the leather, a substance capable of forming with the tannin a compound on which the alcohol has substantially no effect.

4. In the method of making markings on

leather which consists in printing the subject matter on transfer sheet bases with an ink incorporating an alcohol-soluble dye for the leather and vehicle material suiting the ink to the particular printing process by which the printing onto the transfer sheet bases is done and in which vehicle substantially all the dye exists in an undissolved state, and pressing, while the ink vehicle is still present on the transfer sheet, a transfer sheet to the leather in the presence of alcohol, the improvement, where the alcohol tends to have a deleterious affect on the leather, which consists in applying to the leather, at least as early as the time when the alcohol is applied to the leather, a substance forming with the tannin of the leather a compound which is unaffected by the alcohol.

5. The method of making markings on leather which is deleteriously affected by alcohol, which consists in printing the subject matter on transfer sheet bases with an ink incorporating an alcohol-soluble dye for the leather and vehicle material suiting the ink to the particular printing process by which the printing onto the transfer sheet bases is done, and in which vehicle substantially all the dye exists in an undissolved state, applying as a unit to the ink on one of said transfer sheets, while the ink vehicle is still present thereon, a solvent for the dye capable of carrying dye from the ink vehicle into dyeing relation to the fibres of the leather and a substance forming with the tannic acid of the leather a compound which is unaffected by the alcohol, and then pressing the transfer sheet to the leather.

6. The method of making markings on leather which is deleteriously affected by alcohol attacking tannin therein, which consists in printing the subject matter on transfer sheet bases with an ink incorporating an alcohol-soluble dye for the leather and vehicle material suiting the ink to the particular printing process by which the printing onto the transfer sheet bases is done and in which vehicle material substantially all the dye exists in an undissolved state, applying as a unit to the leather alcohol and a substance capable of forming with the tannin of the leather a compound which is substantially unaffected by the alcohol, and pressing, while the ink-vehicle is still present on the transfer sheet and the leather is still wet with said alcohol, a transfer sheet to a wet surface of the leather.

7. The method of making markings on leather which is deleteriously affected by alcohol acting on tannin therein, which consists in printing the subject matter on transfer sheet bases with an ink incorporating an alcohol-soluble dye for the leather and vehicle material suiting the ink to the particular printing process by which the printing onto the transfer sheet bases is done and

in which substantially all the dye exists in an undissolved state, applying alcohol and calcium bromide, and pressing, while the ink-vehicle is still present on the transfer sheet, the transfer sheet to the leather in the presence of the alcohol.

8. The method of making markings on leather which is deleteriously affected by alcohol acting on tannin therein, which consists, in printing the subject matter on transfer sheet bases with an ink incorporating an alcohol-soluble dye for the leather and vehicle material suiting the ink to the particular printing process by which the printing onto the transfer sheet bases is done, and in which substantially all the dye exists in an undissolved state, applying ethyl alcohol and calcium bromide, and pressing, while the ink-vehicle is still present on the transfer sheet, the transfer sheet to the leather in the presence of the alcohol.

In testimony whereof, I have signed this specification.

ADOLF SCHUBERT.

25

30

35

40

45

50

55

60